

# United States Patent

Amakasu et al.

[15] 3,648,006

[45] Mar. 7, 1972

[54] **METHOD OF PRESERVING  
MECHANICAL PROPERTIES OF STEEL  
WIRE DURING SPOT WELDING**

[72] Inventors: **Tatuo Amakasu, Tokyo; Takao Yamazaki,  
Fujisawa, both of Japan**

[73] Assignee: **Koushuha-Netsuren Kabushiki Kaisha,  
Tokyo, Japan**

[22] Filed: **Aug. 3, 1970**

[21] Appl. No.: **60,686**

**Related U.S. Application Data**

[62] Division of Ser. No. 781,174, Dec. 4, 1968, Pat. No.  
3,573,418.

[52] U.S. Cl.....**219/58**

[51] Int. Cl.....**B23k 11/00**

[58] Field of Search.....**219/56, 57, 58**

[56]

**References Cited**

**UNITED STATES PATENTS**

1,878,760 9/1932 Cosgrove et al. ....**219/56 X**

*Primary Examiner—J. V. Truhe*

*Assistant Examiner—Hugh D. Jaeger*

*Attorney—Wenderoth, Lind & Ponack*

[57]

**ABSTRACT**

A method for preserving the mechanical properties of steel wire or rod during spot welding of such steel wire or rod to form cages for use in prestressed concrete. The hoop reinforcing wire is, during the winding operation, preheated between a pair of feeders by direct passage of current therethrough to a temperature of from 300°-1000° C. Thereafter the thus heated wire is successively welded to reinforcing rods.

**1 Claims, 6 Drawing Figures**



Patented March 7, 1972

3,648,006

2 Sheets-Sheet 1

FIG. 1a



FIG. 1b



FIG. 3



TATUO AMAKASU and  
TAKAO YAMAZAKI, Inventors

By *Walter L. P. Brack*  
Attorneys

Patented March 7, 1972

3,648,006

2 Sheets-Sheet 2

FIG. 2a



FIG. 2b



FIG. 4



TATUO AMAKASU and  
TAKAO YAMAZAKI, Inventors

BY, *Wendell L. Bonack*  
Attorneys

**METHOD OF PRESERVING MECHANICAL PROPERTIES  
OF STEEL WIRE DURING SPOT WELDING**

This application is a division of application, Ser. No. 781,174, filed Dec. 4, 1968, now U.S. Pat. No. 3,573,418.

**BACKGROUND OF THE INVENTION**

The present invention relates to a method of preserving the mechanical properties of steel reinforcing wire or rod during spot welding, by preventing deterioration or recovering the lost mechanical properties of the welded parts of said steel wire or rod. More particularly, this invention relates to a method for preserving, by recovering, or preventing loss of, mechanical properties of the welded parts of steel reinforcing wire or rod used in the formation of steel wire cages to be embedded in concrete for the purpose of enhancing the strength of concrete structural products such as concrete pipes, poles, piles, tanks, etc., of prestressed concrete. Such loss of properties occurs when spot-welding the contacting parts of steel rods and hoop-reinforcing wires, said steel rods being arranged parallel to each other and at certain intervals according to the external shape of the concrete structure, and said hoop-reinforcing wires being fixed spirally on the outer circumference of said steel rod arrangement.

Hitherto, in manufacturing prestressed concrete structures, the method which has been generally adopted is to arrange the required number of reinforcing steel rods parallel to each other and at certain intervals, according to the external shape of the structure, such as a concrete pillar or the like which will have the rods incorporated therein. Then steel reinforcing wires or the like are wound spirally around the outer circumference of the steel rod group thus formed.

To fix and secure the contacting parts of said steel rods and said hoop-reinforcing wires, they are bound manually with fine steel wires, thus forming a columnar steel wire cage. Said cage is set in the concrete mold in the proper position, and tension is applied to said steel reinforcing rods while concrete is poured into the mold. This is followed by introducing the necessary stress into the concrete with the steel rods and placing the mold in a centrifugal pillar manufacturing machine or the like to string it up. It is then cured in steam, and the mold is removed. It is then cured in water and in air, and a prestressed concrete pillar is obtained having satisfactory strength and into which the stress has been introduced by the steel rods.

An automatic forming machine has recently been introduced to make highly efficient the production of such a steel reinforcing wire cage that is an essential element for enhancing the strength of such a concrete product.

The object of this invention lies mainly in making it possible to form advantageously and with high efficiency steel wire cages composed of reinforcing steel rods, which cages have excellent mechanical properties.

Other objects and advantages of the invention and its valuable characteristics will become apparent from the following description taken in connection with the accompanying drawings.

**BRIEF DESCRIPTION OF THE DRAWINGS**

FIGS. 1a and 1b are side and end elevation views, respectively, showing a steel reinforcing wire cage;

FIGS. 2a and 2b are graphs showing changes in the mechanical properties of steel reinforcing rods before and after the spot welding of the contacting parts of the hoop-reinforcing wires to said steel rods; FIG. 2a showing the change in tensile strength, and FIG. 2b showing the elongation;

FIG. 3 is a schematic view of one embodiment of heating means for carrying out the method of the invention; and

FIG. 4 is a schematic end view of a form of steel reinforcing wire cage which can be formed successfully by the means shown in FIG. 3.

The above described efficient method of forming steel reinforcing rod cages by using an automatic forming machine will be illustrated with reference to FIG. 1. The required number of steel reinforcing rods 1 are arranged parallel to each other

with their ends fixed to a holding means such as an anchor plate 5. At spaced points along the rods there is positioned within the inner circumference of the rods a drum 4 or the like. The group of steel rods can move and revolve continuously along the outer circumference of said drum 4. Around the outer circumference of the group of steel rods is spirally wound hoop-reinforcing wires 2 made of steel. This is done by relatively rotating the rods and the wire, i.e., by fixing the group of steel rods and rotating the hoop-reinforcing wires 2, or vice versa. The points 3, where the respective steel rods 1 and the hoop-reinforcing wires 2 contact each other, are successively and automatically spot-welded by an electrode 6 for spot welding, which electrode is connected to a power source E.

The rods generally are of a steel having a carbon content of from 0.2-0.65. Typical compositions fall within the ranges of Table I.

TABLE I

| C        | Si       | Mn        | P      | S      |
|----------|----------|-----------|--------|--------|
| 0.2-0.65 | 0.15-2.5 | 0.60-0.90 | <0.030 | <0.035 |

Typical compositions of the hoop-reinforcing wires are shown in Table II.

TABLE II

| C            | Si          | Mn          | P            | S             |
|--------------|-------------|-------------|--------------|---------------|
| 0.15% & less | 0.3% & less | 0.6% & less | 0.69% & less | 0.060% & less |

In so far as formation of this kind of steel wire cage by this method is extremely efficient, said method is superior in comparison to conventional methods. However, a serious shortcoming of said method is that, when the rods 1 and wire 2 are welded, the mechanical properties of the welded parts of the rods deteriorate because said welded parts of the steel rods are suddenly heated and suddenly cooled off.

According to the experimental results obtained by applicants in this respect, the values of the tensile strength and elongation of steel reinforcing rods 1 which have not been spot welded are as indicated by dots c in FIGS. 2a and 2b, respectively, while the values of the tensile strength and elongation of the same steel rods measured after the hoop-reinforcing wires 2 are mechanically separated from the steel rods 1 after having been spot welded thereto is indicated by dots d in the same Figs. As can be seen, the mechanical properties of the steel reinforcing rods 1 will be changed so that the tensile strength will be reduced about 2 percent, and the elongation will be reduced about 50 percent. These reductions were substantially similar to those obtained in other experiments of the same kind. According to the results of applicants' research and experiments, this can be attributed to the fact that a partial metallographical-structural change is brought about in the welded parts of the steel reinforcing rod which contains carbon in an amount up to the level of medium carbon steel. The change in the metallographical structure of the welded portion is due to the fact that it is heated suddenly and quickly by the heat generated during spot welding, and thereafter is suddenly and quickly cooled off. A serious consequence of such a structural change is that it will, in its turn, adversely influence the full achievement of the purpose of this kind of steel wire cage by failure to introduce sufficient stress into the concrete structure to enhance the strength thereof.

After all of the various experiments and studies carried out in an attempt to find a solution to this difficulty, applicants have finally discovered that the hoop-reinforcing wire in the

winding operation should be preheated between a pair of feeders by direct passage of current therethrough to a temperature of from 300° to 1000° C., and then the thus heated wire should be welded to the reinforcing rods at successive spots therealong. By this means, deterioration of the mechanical properties in said welded parts can be effectively prevented.

In FIG. 3 there is schematically shown an apparatus for carrying out the method by direct electrification of the hoop-reinforcing wire, and in which the steel reinforcing rods 1 are surrounded by hoop-reinforcing wire 2. An electrode 6 for spot welding bears on the wire 2 and also serves to press the hoop-reinforcing wires against steel rods 1. A transformer TH for direct electrification has one end of its secondary winding connected electrically to a feeder 7 which is nearer the hoop-reinforcing wire 2 and which is shiftable along said hoop-reinforcing wire 2 and has the other end connected electrically to another feeder 7' having a similar construction. A transformer TW for spot welding has one end of the secondary winding connected electrically to the electrode 6 and the other end connected to the drum 4.

In operation, current from the transformer TH for direct electrification is passed through the feeders 7 and 7' to the hoop-reinforcing wire 2 prior to spot welding them to the steel rods 1 and the hoop-reinforcing wire 2, the current flowing from the feeder 7 through the hoop-reinforcing wire 2 to the feeder 7'. As a result, it is possible to heat the portion of the hoop-reinforcing wire between the feeders 7 and 7' to the required temperature of from 300° to 1,000° C. In this way, the hoop-reinforcing wire 2 heated to the required temperature will be wound automatically around the circumference of the steel rods by rotation of said steel rods in the direction of the arrow in the drawing and longitudinal movement, either of the rods 1 or the feeders 7 and 7'. The steel rods 1 and the heated hoop-reinforcing wire 2 are spot welded by the electrode 6 where they contact each other.

Experiments show that in the method of the invention, when the hoop-reinforcing wire has been heated to a temperature of from 300° to 1,000° C. before the parts of the steel rods and the hoop-reinforcing wire, which contact each other, are spot-welded, deterioration of the mechanical properties of the welded part is only partial and small, and that such insignificant deterioration is rapidly overcome and the parts returned to normalcy by virtue of the heat retained by the hoop-reinforcing wire.

### EXPERIMENTAL RESULTS

TABLE III

| Preheating of<br>Hoop-Reinforcing<br>Wire | Tensile<br>Load      | Elonga-<br>tion<br>(%) | Breaking<br>Position                                        |
|-------------------------------------------|----------------------|------------------------|-------------------------------------------------------------|
| No-heating.....                           | 9380<br>9400<br>9500 | 3.8<br>6.3<br>6.4      | Spot welded part.<br>Spot welded part.<br>Spot welded part. |
| Heating Temperature<br>About 200° C.....  | 9500<br>9550<br>9500 | 6.9<br>5.6<br>7.5      | Spot welded part.<br>Spot welded part.<br>Spot welded part. |
| Heating Temperature<br>About 300° C.....  | 9570<br>9480<br>9500 | 8.9<br>8.3<br>8.3      | Parallel part.<br>Parallel part.<br>Parallel part.          |
| About 400° C.....                         | 9520<br>9530<br>9500 | 8.8<br>8.6<br>9.0      | Parallel part.<br>Parallel part.<br>Parallel part.          |
| 900° to 1000° C.....                      | 9480<br>9500<br>9480 | 9.8<br>9.0<br>9.2      | Parallel part.<br>Parallel part.<br>Parallel part.          |
| Raw Material (Steel<br>Reinforcing Rods)  | 9500<br>9550         | 9.8<br>9.4             |                                                             |

Table 3 shows a part of the experimental results achieved by using the method of direct electrification, and shows a comparison of the mechanical properties of steel rods of the same material where the hoop-reinforcing wires 2 are spot welded without being heated before spot welding, and wherein they are heated to various heating temperatures before spot welding, respectively.

From the above table it is clear that, if the heating temperatures prior to spot welding are from 300° to 1,000° C., the effect of heating the hoop-reinforcing wires 2 is marked, there being substantially no difference between so-called raw material steel reinforcing rods which have undergone no spot welding so far as tensile strength, elongation and breaking position are concerned. In addition, another effect of the method using heating of the hoop-reinforcing wires is that it is possible to reduce the plastic deformation resistance of the hoop-reinforcing wires 2 by heating them to a temperature of from 300° to 1,000° C. before spot welding, and therefore, particularly when steel wire cages of small diameter are to be formed, the conventional operational difficulty heretofore suffered due to the fact that hoop-reinforcing wires are not easily plastically deformed during the winding round the circumference of the steel rods can be eliminated. It is therefore possible, for example, to form a steel wire cage having a square cross section, as shown in FIG. 4.

Further, it should be noted that the system illustrated in FIG. 3 provides a method for very efficiently preventing deterioration of mechanical properties in steel rods without sacrificing the efficiency of forming steel rod cages. Namely, the hoop-reinforcing wire 2, which is being moved for winding around the periphery of a group of steel rods in the cage-forming process, is heated to specified temperature between the two feeders 7 and 7', and said hoop-reinforcing wire maintained at said specified temperature is spotwelded to said rods during movement. Thus, in the process of cage formation, spot welding of wire to rods as well as prevention of deterioration of mechanical properties in steel rods can be finished in a single step without any loss of efficiency and with a negligible loss of energy. On the other hand, in a conventional cage-forming process, it is common practice to wind a hoop-reinforcing wire around the steel rods while shifting the former at a high speed of 20-100 cm./sec. In such a method, when heating the hoop-reinforcing wire in motion with a flame, the energy is insufficient. When induction heating is used, the equipment cost rises. Thus, both methods are unsatisfactory from a practical standpoint. In contrast thereto, direct electrification, as illustrated in FIG. 3, can heat the hoop-reinforcing wire to the specified temperature simply and efficiently while the rods are moved at such high speed before spot welding.

50 What is claimed is:

1. A method of preventing deterioration of the mechanical properties of the welded parts of steel reinforcing rods due to spot welding during formation of steel wire cages for manufacturing prestressed concrete structures, comprising feeding 55 hoop-reinforcing wire through a pair of feeders and winding it around a series of parallel reinforcing rods arranged in a cylinder to carry out a continuous cage winding operation prior to its being spot welded to the reinforcing rods, feeding a direct current from said feeders through the hoop-reinforcing wire between the feeders for heating the wire to a temperature of from 300° to 1,000° C., the wire being substantially immediately contacted with a reinforcing rod after it leaves the feeder closest to the reinforcing rod, and then welding the thus heated wire to the reinforcing rods at successive spots therealong, whereby the wire is welded while it is still substantially at the heated temperature.

\* \* \* \* \*